

Patented May 24, 1932

1,859,848

# UNITED STATES PATENT OFFICE

JOHN D. RUE, OF MADISON, WISCONSIN; SIDNEY D. WELLS, OF QUINCY, ILLINOIS; AND FRANCIS G. RAWLING, OF MADISON, WISCONSIN; SAID RUE AND SAID RAWLING AS SIGNORS TO ARTHUR M. HYDE, SECRETARY OF AGRICULTURE OF THE UNITED STATES

## PRODUCTION OF FIBROUS PULP FROM VEGETABLE MATERIAL

No Drawing.

Application filed September 3, 1926. Serial No. 133,516.

This invention relates to the treatment of vegetable fibrous material to obtain the fiber portion thereof for use in making paper.

The improvement is of particular importance in making, as a new product, an odorless strawboard suitable for egg crate fillers, and one which will remain odorless under cold storage conditions. Combined with the feature of odorlessness, the product resultant of the procedure defined herein contains an unusually large content of both cellulose, lignin and pentosan, as compared to most strawboard materials.

In the production of paper pulp from cereal straws flax, straw, corn stalks, bagasse, rushes, saw grass and other fibrous vegetable materials by means of digestion or boiling in aqueous solutions at elevated temperatures sodium carbonate has been frequently suggested as a softening or pulping agent. It has been found by experience, however, that when used without the addition of caustic lime or alkali the softening action of sodium carbonate alone is insufficient for practical purposes. The present improvement has taught that when sodium sulphite is used in conjunction with sodium carbonate, the softening action is greater than with the use of either alone or with sodium carbonate equal to the sum of the two, and a product is obtained which can readily be beaten, rubbed or pounded to a condition suitable for paper making, and capable of receiving or dispensing with further chemical treatment. Sodium sulphite has been suggested before as a cooking agent but in all cases, it is supposed to play the leading part and is used in relatively large quantities or in conjunction with caustic alkali. One of the troubles experienced in the use of caustic soda is that this chemical is so active that difficulty has been experienced in distributing small amounts through the vegetable material to be cooked without excessive local action. It has also been suggested that sodium sulphite might

be used with sodium bicarbonate, but with results that show that the bicarbonate increases the normal and undesirable tendency toward the acidity of the batch due partially at least to the liberation of un-neutralized organic acids, which acidity tends to produce an undesired brittleness of the partially cooked product.

This invention is equally applicable to treatment of wood chips and wood fiber as described and claimed in our copending application, Serial No. 127,178, filed August 4, 1926.

One of the features of this invention is in the use of sodium carbonate and with relatively large amounts of this material. For instance excellent results have been obtained by using five parts of carbonate to one of sulphite as with the use of 1.5 parts of sodium sulphite and 7.5 parts of sodium carbonate in the digestion of 100 parts of wheat straw. In the digestion of flax straw eight parts of sodium sulphite and twelve parts of sodium carbonate per 100 parts of straw were satisfactory. Variation in the ratio of sodium sulphite and sodium carbonate can be used but the amount of carbonate should be at least 20% of the sulphite. The amount of either the carbonate or the sulphite, considered alone, is insufficient to complete the necessary softening. Sufficient sodium carbonate is desirable, however, to neutralize the organic acids formed by the hydrolytic action of the sodium sulphite. The neutralization of the acids by the sodium carbonate is indicated by the formation of carbon dioxide during the cooking which may be gradually removed by gassing. The sulphite is thus released for further hydrolysis and small amounts will consequently suffice. The mixture is particularly effective in softening the knots in cereal straws and the like while the stems in between may be softened to a milder degree than is possible with present methods and yet yield a satisfactory product.

The following comparative tables show what proportions of cellulose, lignin and pentosan may be obtained by the process of the present invention as compared to other known processes.

|                                                                  | Cellulose | Lignin | Pentosan |
|------------------------------------------------------------------|-----------|--------|----------|
| Wheat straw                                                      | 56        | 28     | 27       |
| Straw board made from lime cooked straw                          | 60        | 22     | 24       |
| Straw board made from sodium sulphite and carbonate cooked straw | 72        | 25     | 29       |
| Bleached straw pulp from caustic soda cooked straw               | 96        | 2      | 32       |
| Flax straw                                                       | 50        | 24     | 24       |
| Pulp made from sodium sulphite and carbonate cooked flax straw   | 71        | 21     | 22       |

In regard to the amounts of cellulose, pentosan and lignin, the total amount of which may be more than 100%, it may be noted that the chemical structures of all of these substances are not definitely known, and the methods of analysis available are only proximate. When cellulose is determined and the residue, which is thought to be cellulose, is tested for pentosan, the amounts to be found may vary from 3 to 15%. Likewise, some of the pentosan shows up in the lignin test as lignin. Accordingly, in the foregoing statement of the methods of analysis which may be used, the total amount of either of these three materials may add up to as much as from 110% to 125%. This is because the figures are the values given by particular methods of analysis, hereinafter specified. A typical analysis of straw board made from sodium sulphite and sodium carbonate, cooked straw is given in the foregoing table. The test for cellulose was 72%; the test for lignin 25%; and the test for pentosan 29%. In conducting the tests different portions of the sample are used for each test. Certain constituents yield a residue, which is reported as cellulose, and also is reported as furfural phloroglucide which tends to indicate that they are of pentosan structure. Furthermore, certain other constituents yield both the residue with sulphuric acid reported as lignin and also furfural phloroglucide, thus showing pentosan structure. The pulps made by cooking with sodium sulphite and sodium carbonate differ from all the others in that they are over 65% and under 80% cellulose while the lignin is over 20% and the pentosan over 20%. Not only do the pulps obtained differ in the amount of cellulose of which they are constituted but they are free from the objectionable musty odor characteristic of lime cooked straw board when it is moistened or has absorbed moisture from damp air such as is present in cold storage plants. This property renders the former pulps suitable for egg case fillers in the storage of eggs and other food products susceptible to the acquisition of taste from the odor of surrounding objects.

In the operation of the process, the following steps are included. The fibrous vegetable material is charged into a boiler or digestor, after cutting, shredding, or crushing into suitable form, if such mechanical treatment is necessary. If a temperature of 212° F. is to be used, open vessels may be utilized. In the case of cereal straw or flax straw, cutting or shredding is not necessary, although certain advantages may be gained by such treatment. The charge of aqueous cooking solution of sodium carbonate and sodium sulphite is then added, and the contents heated by means of the application of either direct or indirect steam. After steaming sufficiently, the digestor is relieved of pressure by opening a valve, whereupon the hot air, carbon dioxide and steam is allowed to escape. More straw may be added and the operation repeated. When the full charge of straw has been added in successive batches, the final heating is performed. Air and carbon dioxide is allowed to escape from time to time, until the excess pressure over the steam pressure for the temperature indicated is as low as is practical. When a temperature of 260° F. is attained, the cooking is usually completed at the end of about eight hours. The steam in the vessel is then relieved and the contents emptied and beaten, pounded, or rubbed either before or after washing to effect the completion of the product into fibers.

The softened material is in condition particularly well adapted for further treatment by the combined pounding and rubbing action of the rod mill process described and claimed in the copending application of Sidney D. Wells, one of the applicants herein, Serial No. 49,461, and from which the disclosure of this present application has been copied.

The material obtained by the chemical treatment may be distinguished by its chemical analysis, using the following methods.

*Cellulose.*—The cellulose is determined by subjecting the material to alternate treatments with chlorine gas in the presence of water and washing with sodium sulphite solutions under the conditions suggested by Cross and Bevan and described by A. W. Schorger Jour. Ind. and Eng. Chem. 9, (1917) 556. In accordance with this, the following procedure is used. Two grams of air dry pulp in an alundum crucible are extracted three to four hours with a mixture of 67 per cent of benzol and 33 per cent alcohol. After evaporation of the solvent the shavings are thoroughly washed with hot water using the suction pump. The moist pulp is then transferred with a pointed glass rod to a 250 cc. beaker, evenly distributed over the bottom, and subjected to a stream (about forty bubbles per minute for each sample) of water washed chlorine gas for half an hour. The end of the tube delivering the chlorine gas should be

about one-half inch above the pulp. At intervals of six to seven minutes the contents of the beaker are stirred to insure uniformity of chlorination. After the chlorine treatment the pulp is treated with a solution of  $\text{SO}_2$  until the chlorine odor disappears, transferred to the alundum crucible, and washed with hot water. The pulp is again returned with the glass rod to the beaker, and 100 cc. of a two per cent sodium sulphite solution are added and the beaker, covered with a watch glass, placed in a boiling water bath for 30 minutes. The fibers are then transferred to the crucible and washed with water. The above procedure is seldom sufficient to remove all the lignin, so that the treatment with chlorine and subsequent treatment as outlined above is repeated until the fibers are practically a uniform white. The second and following treatments with chlorine should not be longer than 15 to 30 minutes. After all the lignin has been removed the fibers are given a final bleaching by adding 20 cc. of a 0.1 per cent solution of potassium permanganate, allowed to stand 10 minutes and rendered colorless with  $\text{SO}_2$  solution. The fibers are then thoroughly washed with hot water, dilute acetic acid, then with hot water, then with alcohol and finally with ether, and dried for two hours at  $105^\circ \text{ C}$ . in the air oven. After cooling by a desiccator over  $\text{H}_2\text{SO}_4$ , the crucible is weighed in a weighing bottle.

*Pentosan.*—The following method is used for determining pentosans and methyl pentosans. Two grams of air dry pulp are placed in a 250 cc. flask provided with a separatory funnel and attached to a condenser (Fig. II). One hundred cc. of 12 per cent hydrochloric acid (sp. gr. 1.06) is added and the contents of the flask are distilled at the rate of 30 cc. in 10 minutes. The distillate is passed through a small filter before entering the receiver. As soon as 30 cc. of distillate are collected 30 cc. of HCl are added to the distillation flask and the distillation is continued in this manner until 360 cc. of distillate are collected. To the total distillate, add 40 cc. of filtered phloroglucine solution that has been prepared at least a week previously by heating 11 grams of phloroglucine in a breaker with 300 cc. of 12 per cent HCl, and after solution has taken place making up to 1500 cc. with 12 per cent HCl. After addition of the phloroglucine, the solution soon turns greenish black. After standing 16 hours the furfural phloroglucide will have settled to the bottom of the beaker. If a drop of the supernatant liquid gives a pink color with aniline acetate paper the precipitation of the furfural is incomplete. A further amount of phloroglucine solution is then added and the beaker allowed to stand over night as formerly. In no case so far has it

been necessary to use more than 40 cc. phloroglucine solution.

The furfural phloroglucide is filtered, using a tared Gooch crucible having a thick asbestos mat and washed with exactly 150 cc. of water. The crucible is then dried for 4 hours in a water oven and weighed in a weighing bottle.

The crucible is placed in a narrow beaker and 20 cc. of 95 per cent alcohol are added to the crucible. The beaker is then placed in a water bath maintained at  $60^\circ \text{ C}$ . for 10 minutes. The alcohol is removed with a suction pump and the process repeated (usually four or five times) until the alcohol that runs through is practically colorless. The crucible is then dried for 2 hours in the water oven and again weighed. The weight of the residue phloroglucide subtracted from the weight of mixed phloroglucide gives the weight of methyl furfural phloroglucide. From the weights of furfural phloroglucide and methyl furfural phloroglucide obtained the amounts of pentosan and methyl pentosan present in the wood are calculated from the table of Krober and Tollens (Aberhalde's "Hand buch der biochemischen Arbeitsmethoden", Vol. II, pp. 137 and 154). The table for the calculation of pentosans has a range for weights of phloroglucide between 0.030 and 0.300 grams. For weights of phloroglucide outside of these limits Krober gives the following formula:

For weight of phloroglucide "a" under 0.030 gm. pentosans =  $(a + 0.0052) \times .8949$  gm. 103

For weight of phloroglucide "a" over 0.300 gm. pentosans =  $(a + 0.0052) \times 0.8824$ .

For the calculation of methyl pentosan the following formula may be used instead of the table:—

$$\text{Methyl pentosan} = (1.85 \text{ Ph} - 625 \text{ Ph}^2 + 0.0040)$$

Ph. is the weight in grams of methyl furfural phloroglucide. 110

*Lignin.*—The lignin or non-cellulose content of pulp is determined by a modification of the method of Ost and Wilkening, employed in the hydrolysis of cellulose. Two to four grams of air dry pulp are weighed in an alundum thimble, extracted with ether in a soxhlet apparatus for 3 to 4 hours, and dried at  $105^\circ \text{ C}$ . The pulp is then removed from the alundum extraction thimbles, placed in 250 cc. beakers, divided into fine particles and treated with 40 cc. of 72.0 per cent sulphuric acid. The hydrolysis is allowed to proceed for 16 hours at room temperature, with frequent stirring at the beginning of the operation. The resulting solution is transferred to a two liter Erlenmeyer flask diluted to 1570 cc. with distilled water, which makes the concentration of  $\text{H}_2\text{SO}_4$  exactly 3 per cent, and boiled under a reflux condenser for two hours. This 120

causes a coagulation of the suspended particles of lignin, which is then filtered on an alundum crucible, washed thoroughly with hot water, dried and weighed as lignin.

5 After the pulps have been beaten, rubbed, or pounded to their ultimate fibers they may be further purified by chlorination, washing with the spent lyes from the digestion or dilute solutions of caustic soda, sodium carbonate, or sodium sulphite or mixtures thereof, bleaching, acidulation or combinations of these steps and a white pulp suitable for white papers can be obtained. For many purposes, however, further treatment is unnecessary and the unbleached material may be manufactured into paper products with the customary machinery known to the art.

20 In the foregoing description only the use of sodium as a base is mentioned. It is of course obvious that any soluble alkaline carbonate, bicarbonate, sulphite or bisulphite which can be so combined either in the digester or before introduction therein to produce the same or similar conditions may be used.

25 From the foregoing it will be recognized that the invention in this process is not directed toward a complete pulping of the material treated, but rather provides a softened material, uniformly softened throughout the thickness of the particles treated, and which is ready for subsequent treatment, as for example by mechanical separation.

In addition to the before mentioned application of Sidney D. Wells, Serial No. 49,461 filed August 10, 1925, the present application and claims are in part copied from Wells application Serial No. 38,354, filed June 19, 1925.

30 This application is a continuation in part of our application Serial No. 100,685, filed April 8, 1926, Treatment of Wood for Production of Pulp.

We claim:

1. In the production of fibers from vegetable material for use in making paper, the method of softening the material to prepare it for subsequent mechanical separation of the fibers which comprises mildly cooking the vegetable material until softened but not pulped into their ultimate fibers with a chemical agent which consists of a solution of sodium carbonate and sodium sulphite, the former being in quantities sufficient to neutralize the acids formed by the hydrolytic action of the sulphite, and in amounts at least as great as twenty percent of the latter.

2. In the production of fibers from vegetable material for use in making paper, the method of softening the material to prepare it for subsequent mechanical separation of the fibers which comprises mildly cooking the vegetable material until softened but not pulped into their ultimate fibers with a chemical agent which consists of a solution of sodium carbonate and sodium sulphite, the

former being in amounts at least as great as twenty percent of the latter.

3. In the production of fibers from vegetable material for use in making paper, the method of softening the material to prepare it for subsequent mechanical separation of the fibers which comprises mildly cooking the vegetable material until softened but not pulped into their ultimate fibers with a chemical agent which consists of a solution of sodium carbonate and sodium sulphite in which the latter does not exceed ten percent of the weight of the vegetable fibrous material being treated.

4. In the production of fibers from vegetable material for use in making paper, the method of softening the material to prepare it for subsequent mechanical separation of the fibers which comprises mildly cooking the vegetable material until softened but not pulped into their ultimate fibers with a chemical agent which consists of a solution of sodium carbonate and sodium sulphite, these chemicals being in such proportion that the total amount of the soda content as  $Na_2O$  does not exceed ten percent of the vegetable fibrous material and the total amount of the  $CO_2$  in the carbonates is at least twenty percent of the  $SO_2$  in the sulphites.

5. A fibrous pulp testing over 65 percent and less than 80 percent of cellulose and having present pentosan and lignin and produced in the treatment of vegetable fibrous material by mild cooking with a chemical agent consisting of an aqueous solution of an alkaline carbonate and alkaline sulphite and which cooking has been followed by mechanical treatment whereby the fibers were separated into pulp.

6. A fibrous pulp testing over 20 percent pentosan and containing cellulose and lignin and produced in the treatment of vegetable fibrous material by mild cooking with a chemical agent consisting of an aqueous solution of an alkaline carbonate and alkaline sulphite and which cooking has been followed by mechanical treatment whereby the fibers were separated into pulp.

7. A fibrous pulp testing over 20 percent of lignin and having present cellulose and pentosan and produced in the treatment of vegetable fibrous material by mild cooking with a chemical agent consisting of an aqueous solution of an alkaline carbonate and alkaline sulphite and which cooking has been followed by mechanical treatment whereby the fibers were separated into pulp.

8. In the production of fibers from vegetable fibrous material, the method of softening the material to prepare it for subsequent mechanical separation of the fibers which comprises mildly cooking the vegetable material until softened but not pulped into their ultimate fibers with a chemical agent which consists of sodium sulphite in amounts too small

of itself alone to effect the desired softening, combined with an alkaline carbonate material capable of counteracting the acidity normally produced by the action of the sulphite.

9. In the production of fibers from vegetable fibrous material, the method of softening the material to prepare it for subsequent mechanical separation of the fibers which

10 comprises mildly cooking the vegetable material until softened but not pulped into their ultimate fibers with a chemical agent which consists of sodium sulphite in amount too small

15 to of itself alone effect the desired softening, combined with an alkaline carbonate material in amounts capable of counteracting the acidity normally produced by the sulphite and too small to alone effect a softening action.

10. In the production of fibers from vegetable fibrous material the method of softening the material to prepare it for subsequent mechanical separation of the fibers which comprises mildly cooking the vegetable material until softened but not pulped into their ultimate fibers with a chemical agent which

25 consists of a solution of sodium carbonate and sodium sulphite, the former being present in amounts at least as great as fifteen percent of the latter, and the latter not exceeding

30 eight percent of the vegetable fibrous material.

11. In the production of fibers from vegetable material for use in making paper, the method of softening the material to prepare it for subsequent mechanical separation of the fibers which comprises first softening the vegetable fibers by subjecting the vegetable material to a chemical treatment which includes mildly cooking the same until softened

40 but not pulped into their ultimate fibers with a chemical agent which consists of an aqueous solution of an alkaline carbonate and sodium sulphite, the former being present in amounts at least twenty percent of the latter, and

45 thereafter subjecting the material thus chemically treated to a mechanical treatment whereby the fibers are separated.

12. In the production of fibers from vegetable material for use in making paper, the method of softening the material to prepare it for subsequent mechanical separation of the fibers which comprises first softening the vegetable fibers by subjecting the vegetable material to a chemical treatment which includes mildly cooking the same at temper-

55 atures between 212° F. and 340° F. until softened but not pulped into their ultimate fibers with a chemical agent which consists of an aqueous solution of an alkaline carbonate

60 and sodium sulphite, the former being present in amounts at least twenty percent of the latter, and thereafter subjecting the material thus chemically treated to a mechanical treatment whereby the fibers are separated.

13. In the production of fibers from vege-

table fibrous material, the method of softening the material to prepare it for subsequent mechanical separation of the fibers which comprises mildly cooking the vegetable material until softened but not pulped into their ultimate fibers with a chemical agent which consists of sodium sulphite in amounts too small to of itself alone effect the desired softening, combined with an alkaline carbonate material capable of counteracting by the relief of carbon dioxide the acidity normally produced by the action of the sulphite.

14. In the production of fibers from vegetable fibrous material, the method of softening the material to prepare it for subsequent mechanical separation of the fibers which comprises mildly cooking the vegetable material until softened but not pulped into their ultimate fibers with a chemical agent which consists of an alkaline sulphite in amounts too small to of itself alone effect the desired softening, combined with an alkaline carbonate material capable of counteracting by the relief of carbon dioxide the acidity normally produced by the action of the sulphite.

15. In the production of fibers from vegetable fibrous material, the method of softening the material to prepare it for subsequent mechanical separation of the fibers which comprises mildly cooking the vegetable material until softened but not pulped into their ultimate fibers with a chemical agent which consists of sodium bisulphite in amounts too small to of itself alone effect the desired softening, combined with an alkaline carbonate material capable of counteracting by the relief of carbon dioxide the acidity normally produced by the action of sulphite.

16. In the production of fibers from vegetable fibrous material, the method of softening the material to prepare it for subsequent mechanical separation of the fibers which comprises mildly cooking the vegetable material until softened but not pulped into their ultimate fibers with a chemical agent which consists of sodium sulphite in amounts too small to of itself alone effect the desired softening, combined with an alkaline carbonate material in amounts of the latter capable of counteracting the acidity normally produced by the sulphite and too small to alone effect a softening action.

17. In the production of fibers from vegetable fibrous material, the method of softening the material to prepare it for subsequent mechanical separation of the fibers which comprises mildly cooking the vegetable material until softened but not pulped into their ultimate fibers with a chemical agent which consists of an alkaline sulphite in amounts too small to of itself alone effect the desired softening, combined with an alkaline carbonate material in amounts of the latter capable of counteracting the acidity normally

produced by the sulphite and too small to alone effect a softening action.

18. In the production of fibers from vegetable fibrous material, the method of softening the material to prepare it for subsequent mechanical separation of the fibers which comprises mildly cooking the vegetable material until softened but not pulped into their ultimate fibers with a chemical agent which 5 consists of sodium bisulphite in amounts too small of itself alone to effect the desired softening, combined with an alkaline carbonate material in amounts of the latter capable of counteracting the acidity normally produced 10 by the sulphite and too small to alone effect a softening action.

19. In the production of fibers from vegetable fibrous material, the method of softening the material to prepare it for subsequent 15 mechanical separation of the fibers which comprises mildly cooking the vegetable material until softened but not pulped into their ultimate fibers with a chemical agent which consists of an alkaline sulphite in amounts 20 too small to of itself alone effect the desired softening combined with an alkaline carbonate, these chemicals being in such proportion that the total amount of alkaline content 25 does not exceed ten percent of the vegetable 30 fibrous material, the total amount of  $\text{CO}_2$  in the carbonates being at least twenty percent of the  $\text{SO}_2$  in the sulphites, and the acidity normally produced by the action of the sulphite being counteracted and controlled 35 by the relief of carbon dioxide formed during the filling and cooking.

20. In the production of fibers from vegetable fibrous material, the method of softening the material to prepare it for subsequent 40 mechanical separation of the fibers which comprises mildly cooking the vegetable material until softened but not pulped into their ultimate fibers with a chemical agent which consists of a sodium sulphite in amounts too 45 small to of itself alone effect the desired softening combined with an alkaline carbonate, these chemicals being in such proportion that the total amount of soda content as  $\text{Na}_2\text{O}$  50 does not exceed ten percent of the vegetable fibrous material, the total amount of  $\text{CO}_2$  in the carbonates is at least twenty percent of the  $\text{SO}_2$  in the sulphites, and the acidity normally produced by the action of the sulphite 55 is counteracted and controlled by the relief of carbon dioxide formed during the filling and cooking.

21. In the production of fiber from vegetable material for use in making paper, the method of softening and separating the fibers 60 which comprises first softening the fibers by subjecting the vegetable material by mildly cooking the same until softened but not pulped into their ultimate fibers with a chemical agent which consists of sodium sulphite 65 in amounts too small to of itself alone effect

the desired softening combined with an alkaline carbonate, these chemicals being in such proportion that the total amount of soda content as  $\text{Na}_2\text{O}$  does not exceed ten percent of the vegetable fibrous material, the total amount of  $\text{CO}_2$  in the carbonates is at least 70 twenty percent of the  $\text{SO}_2$  in the sulphites, and the acidity normally produced by the action of the sulphite is counteracted and controlled by the relief of carbon dioxide 75 formed during the filling and cooking, and thereafter subjecting the fibrous material thus treated to a mechanical treatment whereby the previously softened fibers are separated from each other.

22. In the production of fibers from vegetable material for use in making paper, the method of softening the material to prepare it for subsequent mechanical separation of the fibers which comprises mildly cooking the 80 vegetable material until softened but not pulped into their ultimate fibers with a chemical agent which consists of a solution of sodium carbonate and sodium sulphite, the former being in quantities sufficient to neutralize the acids formed by the hydrolytic 85 action of the sulphite and in amounts approximately five times as great as the latter.

23. In the production of fibers from vegetable material for use in making paper, the method of softening the material to prepare it for subsequent mechanical separation of the fibers which comprises mildly cooking the vegetable material until softened but not pulped into their ultimate fibers with a chemical agent which consists of a solution of sodium carbonate and sodium sulphite the former being in amounts approximately five 90 times as great as the latter.

24. In the production of fibers from vegetable material for use in making paper, the method of softening the material to prepare it for subsequent mechanical separation of the fibers which comprises mildly cooking the vegetable material until softened but not pulped into their ultimate fibers with a chemical agent which consists of a solution of sodium carbonate and sodium sulphite, these chemicals being in such proportion that the total amount of the soda content as  $\text{Na}_2\text{O}$  100 does not exceed ten percent of the vegetable fibrous material and the total amount of the  $\text{CO}_2$  in the carbonates is approximately five times the  $\text{SO}_2$  in the sulphites.

25. In the production of fibers from vegetable fibrous material the method of softening the material to prepare it for subsequent mechanical separation of the fibers which comprises mildly cooking the vegetable material until softened but not pulped into their ultimate fibers with a chemical agent which consists of a solution of sodium carbonate and sodium sulphite, the former being present in amounts approximately five times as 110

great as the latter, and the latter not exceeding 8% of the vegetable fibrous material.

26. In the production of fibers from vegetable material for use in making paper, the method of softening the material to prepare it for subsequent mechanical separation of the fibers which comprises first softening the vegetable fibers by subjecting the vegetable material to a chemical treatment which includes mildly cooking the same until softened but not pulped into their ultimate fibers with a chemical agent which consists of an aqueous solution of an alkaline carbonate and sodium sulphite, the former being present in amounts approximately five times as great as the latter, and thereafter subjecting the material thus chemically treated to a mechanical treatment whereby the fibers are separated.

27. In the production of fibers from vegetable material for use in making paper, the method of softening the material to prepare it for subsequent mechanical separation of the fibers which comprises first softening the vegetable fibers by subjecting the vegetable material to a chemical treatment which includes mildly cooking the same at temperatures between 212° F. and 340° F. until softened but not pulped into their ultimate fibers with a chemical agent which consists of an aqueous solution of an alkaline carbonate and sodium sulphite, the former being present in amounts approximately five times as great as the latter, and thereafter subjecting the material thus chemically softened and loosened to a mechanical treatment whereby the fibers are separated.

28. In the production of fibers from vegetable fibrous material, the method of softening the material to prepare it for subsequent mechanical separation of the fibers which comprises mildly cooking the vegetable material until softened but not pulped into their ultimate fibers with a chemical agent which consists of an alkaline sulphite in amounts too small to of itself alone effect the desired softening combined with an alkaline carbonate, these chemicals being in such proportion that the total amount of alkaline content does not exceed ten percent of the vegetable fibrous material, the total amount of  $\text{CO}_2$  in the carbonates being at least five times as great as the amount of  $\text{SO}_2$  in sulphites, and the acidity normally produced by the action of the sulphite being counteracted and controlled by the relief of carbon dioxide formed during the filling and cooking.

29. In the production of fibers from vegetable fibrous material, the method of softening the material to prepare it for subsequent mechanical separation of the fibers which comprises mildly cooking the vegetable material until softened but not pulped into their ultimate fibers with a chemical agent which consists of a sodium sulphite in amounts too small to of itself alone effect the desired

softening combined with an alkaline carbonate, these chemicals being in such proportion that the total amount of soda content as  $\text{Na}_2\text{O}$  does not exceed ten percent of the vegetable fibrous material, the total amount of  $\text{CO}_2$  in the carbonates is at least five times as great as the  $\text{SO}_2$  in the sulphites, and the acidity normally produced by the action of the sulphite is counteracted and controlled by the relief of carbon dioxide formed during the filling and cooking.

30. In the production of fiber from vegetable material for use in making paper, the method of softening and separating the fibers which comprises first softening the fibers by subjecting the vegetable material by mildly cooking the same until softened but not pulped into their ultimate fibers with a chemical agent which consists of sodium sulphite in amounts too small to of itself alone effect the desired softening combined with an alkaline carbonate, these chemicals being in such proportion that the total amount of soda content as  $\text{Na}_2\text{O}$  does not exceed ten percent of the vegetable fibrous material, the total amount of  $\text{CO}_2$  in the carbonates is approximately five times as great as the  $\text{SO}_2$  in the sulphites, and the acidity normally produced by the action of the sulphite is counteracted and controlled by the relief of carbon dioxide formed during the filling and cooking, and thereafter subjecting the fibrous material thus treated to a mechanical treatment whereby the previously softened fibers are separated from each other.

31. In the production of fibers from vegetable material for use in making paper, the method of softening the material to prepare it for subsequent mechanical separation of the fibers which comprises mildly cooking the vegetable material until softened but not pulped into their ultimate fibers with a chemical agent which consists of a solution of an alkaline carbonate and an alkaline sulphite, the amount of carbonate being approximately five times as great as the amount of sulphite present.

In testimony whereof, we affix our signatures.

JOHN D. RUE.

SIDNEY D. WELLS.

FRANCIS G. RAWLING.

115

120

125

130